

## UNITED STATES PATENT OFFICE

GEORGE C. HALE, OF DOVER, NEW JERSEY

## PROPELLANT POWDER

No Drawing.

Application filed March 1, 1932. Serial No. 596,164.

(GRANTED UNDER THE ACT OF MARCH 3, 1883, AS AMENDED APRIL 30, 1928; 370 O. G. 757)

The invention described herein may be manufactured and used by or for the Government for governmental purposes, without the payment to me of any royalty thereon.

5 This invention relates to a propellant powder.

Modern propellant powders, in addition to being smokeless, are required to be non-hygroscopic, non-volatile and flashless. These 10 additional requirements make much more difficult the formulation of compositions which will also meet ballistic requirements. In the past, there have been two essential types of smokeless powders, the straight 15 nitrocellulose powder containing a volatile solvent as colloidizing agent, and double base powders in which nitrocellulose is colloidized with nitroglycerine. The first type of powder composition mentioned has appreciable 20 volatility, is very hygroscopic and produces a large flash at the muzzle of guns. The nitroglycerine-nitrocellulose powders on the other hand are relatively non-volatile and non-hygroscopic but are not superior to the 25 straight nitrocellulose type in regard to the flash produced.

One means of reducing the flash from nitrocellulose powders is to incorporate inert compounds in the powder. The decomposition 30 of these inert compounds consumes sufficient heat that the temperature of the gases issuing from the muzzle of the gun is reduced below the ignition temperature of the gases and hence no flash is produced. This 35 is a very satisfactory means of reducing flash but it has limitations in other directions in that the addition of inert compounds may reduce the potential of the powder to such an extent that the desired ballistics cannot be 40 obtained.

It would be highly desirable to have a compound available which would act as a colloidizing agent for nitrocellulose and at the same time provide a powder which would be 45 non-hygroscopic, non-volatile, smokeless and flashless. Certain nitroaromatic compounds have been employed in the past in an attempt to provide such a powder but distinct weaknesses can be cited against the use of any of 50 such compounds employed in the past if

judged by their suitability in fulfilling all the requirements of the powder set forth above. Thus, all mononitro compounds employed in the past, while imparting favorable properties such as non-hygroscopicity, non-volatility and a certain tendency to reduce flash, have the objectionable feature of being practically inert and reducing the energy content of the powder in proportion to the amount used. The dinitroaromatic compounds which have been used in propellant powders are crystalline bodies and are, therefore, not colloidizing agents for nitrocellulose at ordinary temperatures. In addition, although they impart greater potential to a 55 powder than the mononitro compound, they have less potential than pyrocellulose and their use with the latter must, therefore, of necessity, reduce the potential of a powder 60 in proportion to the percent used in a basic 65 nitrocellulose composition. The trinitro compounds which have been used have the high potential desired but they are crystalline and hence are not colloidizing agents for nitrocellulose at the temperatures at which 70 powders are manufactured and do not function as well as desired in reducing the hygroscopicity of a powder or in reducing the 75 flash.

Thus, past experience has not yielded a 80 single compound which, when added to nitrocellulose, will give a powder composition that will meet to a satisfactory degree all the requirements now demanded. I have discovered however, a means of accomplishing 85 this end by providing mixtures of nitro compounds which are liquids at ordinary temperature; which have a higher nitrogen content, i. e., potential than any single liquid nitro compound; which impart the properties 90 of non-volatility, non-hygroscopicity and flashlessness to nitrocellulose powders. These mixtures are distinctly superior in this regard to any nitro compound that has previously been used with propellant powders 95 in that these essential requirements are met without detracting appreciably from the energy content or potential of the nitrocellulose. They are, in effect, double base powders in which the objectionable features of 100

nitroglycerine have been eliminated by substituting a liquid mixture of nitro compounds for nitroglycerine.

Examples of compositions which have been prepared and demonstrated by firing tests and chemical tests to meet the requirements mentioned above are cited as follows:

|                      | Per cent |
|----------------------|----------|
| 10 a. Nitrocellulose | 85       |
| 10 Trinitrotoluene   | 5        |
| 10 Mononitrobenzene  | 10       |
| 15 b. Nitrocellulose | 80       |
| 15 Trinitrotoluene   | 15       |
| 15 Mononitrobenzene  | 5        |

15 As a general proposition it may be stated that the TNT may be present in amounts from 5 to 15% and the mononitrobenzene in amounts from 2 to 10%.

20 The advantage of mononitrobenzene over the mononitro compounds of toluene, xylene and naphthalene resides in the fact that it contains a lower percentage of carbon and a higher percentage of oxygen. The benzene 25 molecule contains only six carbon atoms while toluene contains seven, xylene contains eight and naphthalene contains ten.

I claim:

30 A propellant powder consisting of nitrocellulose, trinitrotoluene 5 to 15 per cent and mononitrobenzene 2 to 10 per cent.

GEORGE C. HALE.